

# UNITED STATES PATENT OFFICE.

HENRI ETIENNE ALFRED VITTENET, OF VILLEFRANCE-SUR-SAÔNE,  
FRANCE.

## MANUFACTURE OF ARTIFICIAL SILK AND OTHER SILK GOODS.

No. 842,125.

Specification of Letters Patent.

Patented Jan. 22, 1907.

Application filed July 19, 1905. Serial No. 270,426.

*To all whom it may concern:*

Be it known that I, HENRI ETIENNE ALFRED VITTENET, chemist, a citizen of the French Republic, residing in Villefrance-sur-Saône, Rhône, France, have invented certain new and useful Improvements in the Art of Manufacturing Artificial Silk, of which the following is a specification.

This invention relates to the production of fibers or filaments of artificial silk; and it has for its object to produce a brilliant and supple or flexible filament from a viscous solution of nitrocellulose in acetone.

A solution of pyroxylin or nitrocellulose in acetone yields a viscous collodion which resembles in appearance alcohol-ether collodion and which can be equally well formed in a known way into filaments or threads. The filaments, however, from the solution of pyroxylin in acetone do not possess the brilliancy and suppleness of those from the alcohol-ether collodion, but, on the contrary, are rather opaque, milky, or clouded and are far more brittle than the filaments of the latter. These defects appear to be due to a hydrate of a mixture of the acetone and nitrocellulose.

The purpose of the present invention is to remedy this defect of opacity and brittleness and to provide also for the easy recovery of the acetone. To this end I utilize in carrying out my invention sulfurous acid to prevent hydration, and thus permit of the production of filaments or threads from the viscous compound which will be brilliant and supple or flexible. The sulfurous acid may be employed in several ways, either of which will accomplish the object sought. For example, a suitable quantity of sulfurous acid may be dissolved in the acetone prior to its ultimate employment as the solvent, and when the filaments are formed from the viscous compound they may be produced in the air, in air mixed with sulfurous-acid gas, or in atmosphere formed of sulfurous acid alone, or a solution of pyroxylin in substantially pure acetone in a viscous state may be formed into filaments in an atmosphere of sulfurous-acid gas. The object is to treat the viscous compound in some convenient manner with sulfurous acid to produce the desired effect thereon.

A suitable and convenient mode of carry-

ing out the invention in practice is to cause a current of sulfurous acid to flow into the acetone until an increase in the weight of the mixture is attained which shall be equal to the amount of the acid which it is desired to add to the acetone. The solution of sulfurous acid in acetone thus obtained is then added to the pyroxylin in proportions which will vary with the degree of viscosity desired, and this mixture is formed into filaments, as hereinbefore explained.

Sulfurous-acid gas is employed because it gives to the filaments the required brilliancy, translucency, and suppleness and because it permits of or facilitates the recovery of the acetone. To this end I may produce the filaments of the acetonate collodion in a current of sulfurous-acid gas. It will suffice in order to recover the acetone to heat the combination of gases drawn off in an excess of soda and to properly rectify the aqueous acetone thus obtained.

The acetone employed for dissolving the pyroxylin will be by preference commercial acetone substantially pure.

Having thus described my invention, I claim—

1. The improvement in the art of producing filaments from a viscous solution of pyroxylin and acetone, which consists in forming the said filaments in the presence of sulfurous acid.

2. The improvement in the art of producing filaments from a viscous solution of pyroxylin and acetone, which consists in adding sulfurous acid to the acetone to be used in making the solution, for the purpose specified.

3. The improvement in the art of producing filaments from a viscous solution of pyroxylin in acetone, which consists in adding sulfurous acid to the acetone, then dissolving the pyroxylin therein, and then producing filaments from the solution in an atmosphere containing sulfurous acid.

In witness whereof I have hereunto signed my name, this 28th day of June, 1905, in the presence of two subscribing witnesses.

HENRI ETIENNE ALFRED VITTENET.

Witnesses:

MARIN VACHON,  
PAUL VEYRE.